

# UNITED STATES PATENT OFFICE.

FRANK L. DRIVER, JR., OF NEWARK, NEW JERSEY, ASSIGNOR TO DRIVER-HARRIS COMPANY, OF HARRISON, NEW JERSEY, A CORPORATION OF NEW JERSEY.

## ELECTRIC-RESISTANCE ELEMENT AND ALLOY THEREFOR.

1,321,294.

Specification of Letters Patent.

Patented Nov. 11, 1919.

No Drawing.

Application filed February 7, 1919. Serial No. 275,648.

To all whom it may concern:

Be it known that I, FRANK L. DRIVER, Jr., a citizen of the United States, residing at city of Newark, county of Essex, State of New Jersey, have invented certain new and useful Improvements in Electric-Resistance Elements and Alloy Therefor, of which the following is a full, clear, and exact description.

10 My invention relates to a new and improved electrical resistance element and an alloy therefor, and has for its object to provide a durable resistance element composed of a high heat resisting alloy having a high 15 specific resistance resulting from the presence of substantial quantities of manganese and being of a permanent and uniform character. Heretofore it has been known that the addition of substantial quantities of 20 manganese to a nickel-iron alloy resulted in a marked increase in specific resistance. The nickel-iron-manganese alloy so formed was, however, very difficult to manufacture into uniform resistance elements for the 25 reason that during the various annealings of the metal for the purpose of enabling it to be drawn into wires or rolled into plates the manganese therein oxidized more or less so that the amount of manganese remaining in 30 the alloy after it had been formed into wire or plate was uncertain and indefinite and the specific resistance varied in a corresponding manner. Furthermore, the manganesees of such an alloy oxidizes when the 35 element is heated to a high heat while in use so that after the element has been formed its resistance during use becomes lower in the course of time on account of such oxidation.

I have discovered that by adding to the 40 nickel-iron-manganese alloy a small per cent. of chromium the oxidation and loss of the manganese is practically prevented, the chromium acting as a stabilizer to stabilize the manganese not only during the time 45 when the alloy is being worked into form but also when it is being subjected to high temperatures in ordinary use. For this purpose I have found that between one per cent. (1%) and two per cent. (2%) of 50 chromium is sufficient, and that when chromium to that extent is present in the iron-manganese-nickel alloy above referred to the manganese is well stabilized. In this way a resistance element having a high specific resistance which is permanent in its

character both during the working stage and during the period of use is obtained. The resistance element is also one which is very refractory in its character so that it has a long life even when highly heated. In 60 making the above alloy I make the nickel content about fifty per cent. (50%), there being a zone in the neighborhood of fifty per cent. (50%) nickel and extending from about forty-five per cent. (45%) to fifty-five per cent. (55%) in which considerable variations in the amount of nickel do not produce substantial variations in resistance. The remainder of the alloy in addition to the nickel, manganese and chromium is iron, 70 except for what may be considered as impurities.

In my alloy the specific resistance depends largely upon the amount of manganese present in the alloy. The percentage of 75 manganese should be at least eight per cent. (8%) and I preferably use about ten per cent. (10%), although it may be increased to about twelve (12) or fourteen (14) per cent. Variations from eight per cent. (8%) to 80 fourteen per cent. (14%) of manganese do not cause substantial changes in the specific resistance of the alloy produced, there being a zone within those limits in which the resistance due to the manganese content is 85 approximately constant. As the manganese increases from fourteen per cent. (14%) to eighteen per cent. (18%) the resistance rises quite rapidly and at about twenty per cent. (20%) the alloy becomes so brittle as to be 90 unworkable. In commercial manufacture the resistance obtained by manganese between eight per cent. (8%) and fourteen per cent. (14%) is sufficiently high for most purposes, and I therefore try to make the manganese content about ten per cent. (10%) so as to be sure to have it within the above described zone of substantially fixed resistance. 95

An alloy containing 10.02 per cent. manganese, 1.39 per cent. chromium, 51.10% 100 nickel and the balance of iron constitutes an embodiment of my invention suitable for manufacture of resistance elements for domestic heating devices or similar relations where the temperature of the element 105 when in use does not exceed 1500° F. The silicon should be kept as low as possible and the carbon should preferably not exceed .25 per cent. Cobalt may be substituted for the nickel, it being well known that these two 110

metals have common characteristics, and where I refer to a metal having the characteristics common to nickel or cobalt, I mean to refer to either of those metals.

The alloy whose composition I have specifically referred to above has a resistance of between 600 to 660 ohms per circular mil foot. It can be melted in either crucible or electric furnaces, cast into ingots, worked down under the hammer, rolled to wire rod by a hot process and drawn cold through dies. It is malleable and ductile, and can be drawn into very fine wire in a commercial manner.

15 In producing my alloy I preferably use an electric furnace the charge being made up so as to have the proper portions in the alloy and melted in the ordinary manner.

As will be evident to those skilled in the art, my invention permits of various modifications without departing from the spirit thereof or the scope of the appended claims.

What I claim is:

1. An alloy comprising substantial proportions of iron, manganese, chromium and a metal having the characteristics common to nickel and cobalt, the percentage of the last named element lying within the approximately constant resistance zone including nickel fifty per cent. (50%), the percentage of the manganese lying within the approximately constant resistance zone including manganese ten per cent. (10%), and the percentage of chromium being low.

35 2. An alloy comprising substantial proportions of iron, manganese, chromium and a metal having the characteristics common to nickel and cobalt, the percentage of the last named element being between forty-

40 five per cent. (45%) and fifty-five per cent. (55%), the percentage of the manganese being between eight per cent. (8%) and fourteen per cent. (14%) and the percentage of chromium being less than half of the manganese.

45

3. An alloy comprising iron, manganese, chromium and a metal having the characteristics common to nickel and cobalt, the percentage of the last named element being between forty-five per cent. (45%) and fifty-five per cent. (55%), the percentage of the manganese being between eight per cent. (8%) and fourteen per cent. (14%) and the percentage of chromium being between one per cent. (1%) and two per cent. (2%).

55

4. An alloy comprising iron, manganese, chromium and a metal having the characteristics common to nickel and cobalt, the percentage of the last named element being about fifty per cent. (50%), the manganese being about ten per cent. (10%) and the chromium about one and five-tenths per cent. (1.5%).

60

5. A resistance element composed of an alloy comprising substantial proportions of iron, manganese, a stabilizer for the manganese consisting of a metal of the chromium group and a metal having the characteristics common to nickel and cobalt, the percentage of the last-named element lying within the approximately constant resistance zone including fifty per cent. (50%), the percentage of manganese lying within the approximately constant resistance zone including ten per cent. (10%) and the percentage of the stabilizer being low.

70

FRANK L. DRIVER, JR.